

H. R. KEITHLEY.  
COMPOUND CAR WHEEL.

APPLICATION FILED MAY 12, 1911. RENEWED JAN. 9, 1915.

1,149,267.

Patented Aug. 10, 1915.

*Fig. 1.*



*Fig. 2.*



*Fig. 3.*



*Fig. 4.*



Witnesses:

*Harry S. Gaither*  
*J. H. Morgan*

Inventor:

*Herbert R. Keithley*  
by *Chamberlain & Gunderson*  
*Atlys*

# UNITED STATES PATENT OFFICE.

HERBERT R. KEITHLEY, OF KANSAS CITY, MISSOURI.

## COMPOUND CAR-WHEEL.

1,149,267.

Specification of Letters Patent. Patented Aug. 10, 1915.

Original application filed April 26, 1909, Serial No. 492,323. Divided and this application filed May 12, 1911, Serial No. 626,668. Renewed January 9, 1915. Serial No. 1,456.

To all whom it may concern:

Be it known that I, HERBERT R. KEITHLEY, a citizen of the United States, residing at Kansas City, county of Jackson, State of Missouri, have invented a certain new and useful Improvement in Compound Car-Wheels, and declare the following to be a full, clear, and exact description of the same, such as will enable others skilled in the art to which it pertains to make and use the same, reference being had to the accompanying drawings, which form a part of this specification.

The object of this invention is to produce a car wheel in which the body portion, comprising the hub and web and a part of the inner portion of the rim, shall be made of low carbon soft steel, having the properties of strength, toughness and great resistance to stresses from shock, and in which the wearing body of the rim and flange shall be made of high carbon hard steel, or a hard steel alloy, preferably of manganese steel having above 6% content of manganese and which shall differ greatly in carbon content, or in metallic composition, from that of the low carbon soft steel forming the body portion, and possesses properties of intense hardness and great resistance to abrasion and wear.

The various features of novelty whereby my invention is characterized will herein-after be pointed out with particularity in the claims; but, for a full understanding of my invention and of its object and advantages, reference may be had to the following detailed description taken in connection with the accompanying drawing, wherein:

Figure 1 is a central transverse section showing the cast blank from which my improved wheel is made in position in the forging dies for reducing the blank to the shape of the car wheel; Fig. 2 is a section similar to Fig. 1, showing the dies closed; Fig. 3 is a side view of one half of the completed wheel; and Fig. 4 is a central transverse section through the wheel.

The first step in the production of my improved wheel is the formation of a suitable cast blank having portions of hard steel and of soft steel united by casting and arranged in such a way as to permit the blank to be forged into the shape of a car wheel with the soft and hard portions distributed in the proper manner. The blank

which I prefer to use is preferably one produced in a specially constructed mold as explained in detail in my application #492,323 for process of manufacturing car wheels, filed April 26, 1909 and which has matured into Patent #1,073,350 of September 16, 1913, of which the present application is a division; the hard steel being first poured into the mold and collecting in the form of an annular ring which becomes the rim of the blank, and the soft steel being then poured on top of the hard steel, completing the rim and forming the center of the blank. After the blank is removed from the mold and the riser is discarded, it has the form shown in Fig. 1; there being a rudimentary hub 1, on one side of the web 2, and an annular flange or rim 3 projecting laterally from the web along the edge thereof. The hub member and the web member are of soft steel and the annular rim or flange 3 lying below the dotted line 4 is made of hard steel.

The riser is preferably removed by punching out the central portion of the hub thereby discarding the pipe and segregations which concentrate toward the center of the casting and rise to the top of the fluid steel as the metal solidifies in the mold.

When the blank is placed between forging dies such as indicated at 5 and 6, and the dies are closed, the hard steel of the rim portion 3 is caused to flow under the pressure of the dies to the outer periphery of the wheel so as to form the wearing body portion of the wheel rim 7 and of the flange 8, as indicated in Figs. 2 and 4; and the soft steel, integrally united with the hard steel in the rim, is caused to flow under the pressure of the dies so as to form the inner portion of the wheel rim and a backing for the wearing body of the flange as indicated by the area 9 lying above the dotted line 10 in Figs. 2 and 4. Consequently the wearing faces of the rim and of the flange are composed of steel of intense hardness which offers great resistance to abrasion and wear, and they are backed and integrally united with a mass of soft tough steel which possesses great strength and offers great resistance to stresses from shock.

The use of manganese steel containing above six per cent. of manganese is made available by this method for forming the wearing body of the rim and flange of a car

wheel embodying my invention, and is preferred for this purpose on account of its qualities of intense hardness and toughness and great resistance to abrasion and wear, 5 also to its further remarkable properties which render it almost impossible to anneal or soften this metal. By heat-treatment it can be made tough and ductile, while still retaining its intense hardness, by sudden 10 cooling from a high temperature, by quenching. Whereas, other hard steels are rendered brittle by the same treatment. However, it is obvious that other high carbon steel or steel alloys may be used for this purpose without departing from the scope of my invention, as set forth in the claims.

In all steel wheels at present produced by forging the wheel into shape, the carbon content and composition of metal is uniform 20 throughout, from the hub to the rim, and on account of its softness and rapid wear in service the wheel rim is made very heavy to allow for wear and for restoring the proper contour to the tread and flange by turning 25 the wheel in a lathe. This involves greater first cost for extra metal in the wheel rim and further expense in repairs and maintenance for wrought steel wheels of this type. Whereas, in a car wheel produced according 30 to my invention the wearing body of the wheel rim can be made much lighter, and the composition of metal can be made such that maximum service can be obtained with greatly reduced wear.

35 In a car wheel produced according to my invention the metal may be subjected to heat-treatment, if required, after the wheel is forged into shape, or the cast blank may be heat-treated before it is forged, or both the cast blank and the forged wheel may be heat-treated if desired.

40 The carbon content of the relatively low carbon soft steel forming the web and hub portions of the cast blank of the wheel, can be so proportioned that heat-treatment with air cooling, water or other quenching found adapted to both the hard steel rim and the soft steel body portion can be used, this being one of the important advantages of my 45 invention.

50 I claim:

1. As an article of manufacture a car-wheel having its body portion, consisting of the hub, the web and inner portion of the 55 rim, composed of low carbon soft steel, and having formed therewith, by forging, a wearing rim and flange portion composed of relatively high carbon hard steel, said soft metal body portion and hard metal rim and flange portion being united integrally in one body of metal by casting.

60 2. As an article of manufacture a car-wheel having its body portion, consisting of

the hub, the web and inner portion of the rim, composed of low carbon soft steel, and having formed therewith, by forging, a wearing rim and flange portion composed of a hard steel alloy, said soft steel body portion and hard steel rim and flange portion being united integrally in one body of metal 70 by casting.

3. As an article of manufacture a car-wheel having its body portion, consisting of the hub, the web and inner portion of the rim, composed of low carbon steel, and having formed therewith, by forging, a wearing rim and flange portion composed of manganese steel, said soft steel body portion and manganese steel rim and flange portion being united integrally in one body of metal 80 by casting.

4. As an article of manufacture, a car-wheel having its body portion, consisting of the hub, the web, the inner portion of the rim and the back of the flange, composed of 85 low carbon soft steel, and having formed therewith by forging, a wearing rim portion and a wearing flange portion composed of relatively high carbon hard steel, said soft metal body portion and hard metal rim and flange portion being united integrally in one body of metal by casting.

5. A car wheel of soft steel having the center of low carbon soft steel and having wearing portions of the flange and rim 95 formed of high carbon steel, the soft steel portion extending outwardly into the flange beyond the tread portion of the rim.

6. A car wheel having its body portion, consisting of the hub, the web, and a continuation of the web through the rim and into the flange composed of low carbon soft steel, and having a ring of hard steel lying beside and integrally united with the soft steel to complete the rim and the flange.

7. A car wheel having a soft steel center and hard steel wearing surfaces for the flange and rim, the soft steel being continued from the web of the wheel out through the flange and forming the back side of the flange.

8. A car wheel having a soft steel center and a rim and flange containing hard steel, the soft steel and the hard steel being united by casting along a surface dividing the rim into two parts, the metal in the wheel body 11 within the space bounded by said surface being substantially homogeneous and the body of hard metal outside of said surface being also substantially homogeneous.

In testimony whereof, I sign this specification in the presence of two witnesses.

HERBERT R. KEITHLEY.

Witnesses:

Wm. F. FREUDENREICH,  
RUBY V. BRYDGES.